

3,510,243

**PROCESS FOR THE CONTINUOUS DYEING AND PRINTING OF FIBRE MATERIAL FROM LINEAR, HIGH MOLECULAR ESTERS OF AROMATIC POLYCARBOXYLIC ACIDS WITH POLYFUNCTIONAL ALCOHOLS**

Marcel Seuret, St. Kilda, Melbourne, Victoria, Australia, and Willi Leutenegger, Bottmingen, Basel-Land, and Hans E. Wegmuller, Riehen, Switzerland, assignors to

J. R. Geigy A.G., Basel, Switzerland

No Drawing. Filed Dec. 1, 1966, Ser. No. 598,184  
Int. Cl. C09b 1/00, 5/62

U.S. Cl. 8—39

13 Claims

**ABSTRACT OF THE DISCLOSURE**

A process for the continuous dyeing or printing of fiber material from linear, high molecular esters of aromatic polycarboxylic acids with polyfunctional alcohols, is provided. There is applied to the fiber material a solution of (A) a mixture of solvents consisting essentially of

- (a) 50 to 99% by weight of a water-insoluble chlorinated hydrocarbon having a boiling point between 50 and 150° C.;
- (b) 50 to 1% by weight of a liquid, water-soluble, organic solvent having a boiling point below 220° C., and
- (B) a dispersion dyestuff, e.g. anthroquinone.

The resulting dyeing or print on the fiber material is then fixed by subjecting the treated fiber material to a subsequent heat treatment at temperatures from about 130° C. to below the softening point of the fiber material.

The present invention concerns a process for the continuous dyeing and printing of fibre material from linear, high molecular esters of aromatic polycarboxylic acids with polyfunctional alcohols, the dye liquor used therefore, as well as the fibre material dyed or printed by this process.

As it is known, linear, high molecular esters of aromatic polycarboxylic acids with polyfunctional alcohols are dyed with aqueous dyestuff dispersions either from a long bath at the boiling point of the water and in the presence of so-called carriers, or at temperatures of 100 to 150° C. under pressure, or by impregnating with an aqueous, thickened dyestuff dispersion, drying, thermofixing the dyestuff on this material and, finally, washing out the thickener and dispersing agent. These dyeing processes, however, have several disadvantages: one is that the dispersion dyestuffs must be brought into a finely dispersed form which necessitates time-consuming milling operations with suitable dispersing agents, and also they cause great amounts of waste water so that comprehensive purification of waste water is necessary.

This led to the idea of dyeing the material mentioned above with organic dyestuff solutions. One suggestion is to treat polyethylene glycol terephthalate films with a solution or dispersion of disperse dyestuffs in a solvent which wets the polyethylene glycol terephthalate and then to subsequently fix the dyestuff on this material by a heat treatment. Methyleneethyl ketone, benzyl alcohol, toluene, methyl isobutyl ketone, anisol, ethyl acetate, cyclohexanone and a mixture of dimethyl acetamide and methylethyl ketone are mentioned as solvents.

This process, however, is unsuitable for the dyeing of polyethylene glycol terephthalate textile material, as generally, dull and weakly coloured dyeings are obtained.

A process has now been found by which fibre material from linear, high molecular esters of aromatic polycar-

boxylic acids with polyfunctional alcohols, particularly polyethylene glycol terephthalate fibres, can be continuously dyed and printed. The new process consists in applying to said fibre material a solution comprising a mixture of solvents consisting essentially of

- (a) 50 to 99 percent by weight of unhalogenated or halogenated hydrocarbon having a boiling point between 50 and 150° C.;
- (b) 50 to 1 percent by weight of a liquid, water-soluble, organic solvent having a boiling point below 220° C., and
- (c) a dispersion dyestuff soluble in said mixture, in a sufficient amount to impart to said fibre material in a desired color depth,

and also, if necessary, a thickener, removing a substantial part of excess dye liquor from the material and fixing the resulting dyeing or print on said fibre material by subjecting the treated fibre material to a subsequent heat treatment at temperatures below the softening point of the fibre material.

Surprisingly deep, brilliant dyeings which are fast to rubbing are obtained by this process without after-soaping thereof. Their brilliancy is completely equal to that of dyeing attained by the usual processes with aqueous dispersions and their depth of shade is, in some cases, even superior. The time consuming milling operations necessary to attain a fine distribution of the dyestuffs are unnecessary. Also, the mixtures of solvents to be used according to the invention can easily be regained and used again in the dyeing process; moreover, in contrast to the previously known processes all refining of waste water becomes superfluous as the after-soaping in rinsing baths which has been usual hitherto is not necessary.

Suitable hydrocarbons boiling between 50 and 150° C. which can be used as component (a) of mixtures of solvents usable according to the invention are, e.g. aromatic hydrocarbons such as toluene or xylene; preferably however, these mixtures of solvents contain 50 to 99 percent by weight of halogenated, particularly chlorinated, hydrocarbons, e.g. chlorobenzene, mainly however, low aliphatic halogenated hydrocarbons such as chlorinated hydrocarbons, e.g. chloroform, carbon tetrachloride, tri- or tetra-chloroethylene ("perchloroethylene"), tetrachloroethane or dibromoethylene. Also mixtures of such solvents can form the water insoluble component of mixtures of solvents usable according to the invention.

By "liquid, water soluble, organic solvents boiling below 220° C." (b) are meant thermostable solvents which are water soluble not only to fractions of percentages but to some percentages. Examples thereof are benzyl alcohol, cyclohexanone, cyclohexanol, n. and sec. butyl alcohol or methylethyl ketone. Preferred, however, are those solvents as defined which are miscible with water in any ratio. Examples thereof are: monovalent low aliphatic alcohols such as, e.g. methanol, ethanol and n- or isopropanol; alkylene glycol monoalkyl ethers such as ethylene glycol monomethyl or monoethyl ether; then also furfuryl alcohol or tetrahydrofurfuryl alcohol; or divalent aliphatic alcohols such as ethylene glycol or 1,2-propylene glycol; also low aliphatic ketones such as acetone; low cyclic ethers such as dioxane; also amides of low fatty acids such as dimethyl formamide or dimethyl acetamide; then carbonic acid amides, such as tetramethyl urea; or tertiary organic amines such as pyridine; as well as mixtures of such organic solvents.

Mixtures of solvents are preferred which consist of 80 to 99 percent by weight of chlorinated lower aliphatic hydrocarbon boiling between 50 and 150° C. and of 20 to 1 percent by weight of an organic solvent boiling below 220° C. which is water-miscible in any ratio. In particular,

mixtures of 90 percent by weight of perchloroethylene or trichloroethylene and 10 percent by weight of methanol or tetrahydrofurfuryl alcohol are suitable.

The composition of the mixture of solvents depends on the solubility of the dyestuff or mixture of dyestuffs to be used. Preferably homogeneous clear dyestuff solutions are used.

Dispersion dyestuffs usable according to the invention can belong to any classes of dyestuffs desired. They are, in particular, metal-free azo dyestuffs, also anthraquinone, nitro, methine, styrene, azostyrene, naphthoperinone, quinophthalone or naphthoquinone imine dyestuffs, which are free from water solubilising groups which dissociate acid in water.

Depending on the desired depth of shade, the dyestuff solution to be used according to the invention contains 0.1 to 10 percent by weight of one or more of the dyestuffs mentioned.

If necessary, the dye solution usable according to the invention can also contain thickeners, advantageously those which are soluble in the defined mixture of solvents, e.g. thickeners having a basis of cellulose ester or polyvinyl alcohol or ester.

The fibre material as defined is impregnated, e.g. by printing or spraying, preferably however, by pad dyeing in the foulard. In the latter case, the fibre material is continuously passed through the dyestuff solution, advantageously at room temperature, then squeezed out to the desired content of impregnation solution of about 30 to 150 percent by weight (calculated on the dry weight of the goods). The main part of the mixture of solvents remaining in the fibre material is then removed, advantageously under mild conditions at 40 to 80° C., particularly in a warm, dry airstream. The dyestuff is then fixed by a subsequent heat treatment on the still moist or optionally already dried fibre material either by steaming, preferably under pressure at about 130° C., or by a dry heat treatment at a temperature of at least 180° C. but below the softening point of the fibre material. These two types of heat treatment can also be combined, but the dry heat treatment, the so-called thermofixing, is preferred. Contact heat, a treatment with high frequency alternating currents or infrared irradiation is suitable for this purpose; preferably, however, the dyestuff is fixed on the fibre material in a hot airstream at 180 to 230° C., particularly at a temperature of 200 to 220° C.

Level, strongly coloured and fast dyeings are obtained on the fibre material mentioned by the process according

to the invention; for example the dyeings are fast to dry cleaning, perspiration and rubbing.

The following examples illustrate the invention. The temperatures are given in degrees centigrade.

### EXAMPLE 1

10 g. of dyestuff of the formula



are dissolved in 1000 g. of a mixture of solvents which consists of 90 percent by weight of perchloroethylene and 10 percent by weight of methanol. The solution is clarified by filtration. Polyethylene glycol terephthalate fabric is impregnated at room temperature with this clear, yellow dye solution, the impregnated fabric is squeezed out to about 100 percent content of solution (calculated on the dry weight of the goods) and dried at 40 to 80° C. The impregnated and dried fabric is then thermofixed for 3 minutes at 220° C.

30 A strongly coloured, level, brilliant and well developed gold-yellow dyeing is obtained.

If, in the above mixture of solvents, the perchloroethylene is replaced by the same amount of toluene or dibromoethylene and otherwise the procedure described in this 35 example is followed, then dyeings of similar quality are obtained.

If, in the above mixture of solvents, the perchloroethylene and methanol are used in a weight ratio of 80:20 instead of 90:10, then with otherwise the same procedure, similar results are obtained.

If, instead of the dyestuff mentioned in the example, the same amount of one of the dyestuffs given in column 40 2 of the following Table I is used and otherwise the procedure given in the example is followed, then strongly coloured, level and well developed dyeings on polyethylene glycol terephthalate are obtained of the shades given in column 3 of this table.

TABLE I

| Example No. | Dyestuff | Shade on poly-<br>ethylene glycol<br>terephthalate |
|-------------|----------|----------------------------------------------------|
| 2           |          | Blue.                                              |
| 3           |          | Red.                                               |
| 4           |          | Bluish red.                                        |
| 5           |          | Violet.                                            |

## Example No. Dyestuff

Shade on poly-  
ethylene glycol  
terephthalate

|     |  |                  |
|-----|--|------------------|
| 6.  |  | Violet.          |
| 7.  |  | Blue.            |
| 8.  |  | Green.           |
| 9.  |  | Reddish yellow.  |
| 10. |  | Orange.          |
| 11. |  | Yellow.          |
| 12. |  | Greenish yellow. |
| 13. |  | Yellow.          |
| 14. |  | Greenish yellow. |
| 15. |  | Blue.            |
| 16. |  | Greenish yellow. |

7  
EXAMPLE 17

5 g. of the dyestuff of the formula



are dissolved in 1000 g. of a mixture of solvents which consists of 85 percent by weight of trichloroethylene and 15 percent by weight of methanol. After clarifying the solution, polyethylene glycol terephthalate fabric is impregnated and dried as described in Example 1. The impregnated and dried fabric is then thermofixed for 90 seconds at 200° C.

A strongly coloured, level and well developed red dyeing is obtained.

If, instead of 85 percent by weight of trichloroethylene, the same amount of perchloroethylene and/or instead of 15 percent by weight of methanol, the same amount of 20 benzyl alcohol is used and otherwise the procedure given in the example is followed, then similar results are obtained.

If the impregnated and dried fabric is not thermofixed but steamed at 130° for 10 minutes under pressure, then 25 similar good results are obtained.

## EXAMPLE 18

7 g. of the dyestuff of the formula



are dissolved in 1000 g. of a mixture of solvents which 35 consists of 90 percent by weight of chloroform and 10 percent of weight of ethanol and this solution is clarified. A polyethylene glycol terephthalate fabric is impregnated with the clear red dye solution and dried as described in Example 1. The impregnated and dried material is 40 then thermofixed for 5 minutes at 190° C.

A level and intensively red dyeing is obtained.

If, instead of chloroform, the same amount of trichloroethylene, perchloroethylene and/or instead of ethanol, the same amount of methanol, tetrahydrofurfuryl alcohol, 45 isopropanol or dimethyl formamide is used and otherwise the procedure given in the example is followed, then dyeings having similar good properties are obtained.

If a mixture of solvents consisting of 50 percent by weight of perchloroethylene and 50 percent by weight of 50 methanol is used and otherwise the procedure given in the example is followed, then a level and intensively red dyeing is also obtained.

## EXAMPLE 19

6 g. of the dyestuff of the formula



are dissolved in 1000 g. of a mixture of solvents which consists of 90 percent by weight of chlorobenzene and 10 percent by weight of methanol and the solution is 65 clarified.

A fabric made from polyethylene glycol terephthalate 70 is impregnated with this clear violet solution and dried as described in Example 1 and thermofixing of the impregnated and dried fabric is then performed for 2 minutes at 210° C.

A level and strongly coloured violet dyeing is obtained. 75

8  
EXAMPLE 20

5 g. of the dyestuff of the formula



are dissolved in 1000 g. of a mixture of solvents which consists of 97 percent by weight of perchloroethylene and 3 percent by weight of dimethyl formamide and the solution is clarified. Polyethylene glycol terephthalate fabric is impregnated with this solution and dried as described in Example 1. The impregnated and dried fabric is then thermofixed for 4 minutes in a hot airstream at 200° C.

A level and strongly coloured violet dyeing is obtained.

If, in the mixture of solvents given above, the dimethyl formamide is replaced by the same amount of ethylene glycol monomethyl or monoethyl ether or by pyridine, then with otherwise the same procedure, similar results are obtained.

## EXAMPLE 21

5 g. of the dyestuff of the formula



are dissolved in 1000 g. of a mixture of solvents which consists of 95 percent by weight of perchloroethylene and 5 percent by weight of dimethyl acetamide and the solution is clarified. A polyethylene glycol terephthalate fabric is impregnated with this solution and dried as described in Example 1. The impregnated and dried fabric is then thermofixed at 200° C. for 90 seconds with an apparatus for infrared irradiation.

A brilliant, level red dyeing is obtained.

We claim:

1. A process for the continuous dyeing or printing of fiber material from linear, high molecular esters of aromatic polycarboxylic acids with polyfunctional alcohols, comprising:

(I) applying to said fiber material a solution consisting essentially of

(A) a mixture of solvents consisting essentially of (a) 50-99 percent by weight of a water-insoluble chlorinated hydrocarbon having a boiling point between 50 and 150° C.;

(b) 50-1 percent by weight of a liquid, water-soluble, organic solvent having a boiling point below 220° C. and selected from the group consisting of monovalent aliphatic alcohols having from 1 to 4 carbon atoms, ethylene glycol monomethyl or monoethyl ether, furfuryl alcohol, tetrahydrofurfuryl alcohol, ethylene glycol, 1,2-propylene glycol, acetone, dioxane, dimethyl formamide, dimethyl acetamide, tetramethyl urea, pyridine, benzyl alcohol, cyclohexanone, cyclohexanol or methylethyl ketone, or mixtures of these solvents, and

(B) a dispersion dyestuff, and

(II) fixing the resulting dyeing or print on said fiber material by subjecting the treated fiber material to a subsequent heat treatment at temperatures from about 130° C. to below the softening point of the fiber material.

2. A process as described in claim 1, wherein said component (a) is a chlorinated lower aliphatic hydrocarbon having a boiling point between 50 and 150° C.

3. A process as described in claim 1, wherein said component (a) is perchloroethylene or trichloroethylene.

4. A process as described in claim 1, wherein said component (b) is methanol or tetrahydrofurfuryl alcohol.

5. A process as described in claim 1, wherein said dispersion dyestuff is a metal-free azo dyestuff.

6. A process as described in claim 1, wherein said dispersion dyestuff is an anthraquinone dyestuff.

7. A process as described in claim 1, wherein said dispersion dyestuff is a nitro dyestuff.

8. A process as described in claim 1, wherein said dispersion dyestuff is a styrene dyestuff. 5

9. A process as described in claim 1, wherein said dispersion dyestuff is a naphthoquinoneimino dyestuff.

10. A process as described in claim 1, wherein in step (I) said fiber material is impregnated with said non-aqueous solution. 10

11. A process as described in claim 1, wherein in step (II) said dyeing is fixed by heat treating the impregnated fiber material in dry air at a temperature of from at least 180° C. to a temperature below the softening point of 15 the fiber material.

12. A process as described in claim 1, wherein said fiber material consists essentially of polyethylene glycol terephthalate fibers.

13. Fiber material from linear, high molecular esters 20 of aromatic polycarboxylic acids with polyfunctional alcohols, dyed or printed by the process described in claim 1,

## References Cited

## UNITED STATES PATENTS

2,274,751 3/1942 Sowter et al. ----- 8—94 X  
3,129,053 4/1964 Castle ----- 8—93

## FOREIGN PATENTS

917,925 2/1963 Great Britain.

## OTHER REFERENCES

L. Diserens, The Chemical Technology of Dyeing and Printing, vol. II, pp. 207—209, 1951, Reinhold Publ. Corp., New York.

GEORGE F. LESMES, Primary Examiner

T. J. HERBERT, Jr., Assistant Examiner

U.S. CL. X.R.

8—41, 83, 94, 172, 174, 175, 179